

R. F. BACON AND H. S. DAVIS.

TREATMENT OF MINED SULFUR.

APPLICATION FILED OCT. 6, 1919.

1,374,898.

Patented Apr. 19, 1921.



Inventors:

Raymond F. Bacon,  
Harold S. Davis,

By their Attorneys,  
Fannie Davis, Stuart Edwards.

# UNITED STATES PATENT OFFICE.

RAYMOND F. BACON AND HAROLD S. DAVIS, OF PITTSBURGH, PENNSYLVANIA,  
ASSIGNORS TO TEXAS GULF SULPHUR COMPANY, OF BAY CITY, TEXAS, A  
CORPORATION OF TEXAS.

## TREATMENT OF MINED SULFUR.

1,374,898.

Specification of Letters Patent. Patented Apr. 19, 1921.

Application filed October 6, 1919. Serial No. 328,935.

To all whom it may concern:

Be it known that we, RAYMOND F. BACON, a citizen of the United States, and HAROLD S. DAVIS, a citizen of the Dominion of Canada, both residing in Pittsburgh, Allegheny county, State of Pennsylvania, have invented certain new and useful Improvements in the Treatment of Mined Sulfur, (Case B;) and we do hereby declare the following to be a full, clear, and exact description of the invention, such as will enable others skilled in the art to which it appertains to make and use the same.

In an application filed of even date herewith, we have described a method for improving the free burning properties of mined sulfur, by maintaining a molten body of the sulfur at a temperature sufficient to carbonize the oil contained therein.

The present application contemplates not only the carbonizing of the oil by the method referred to, but also the elimination of the carbon from the sulfur, so that the final product shall be of a grade comparable to and useful for purposes for which refined sulfur is now employed in the arts.

In carrying out the invention, the mined sulfur, as fully described in our application hereinbefore referred to, is delivered into a receptacle (preferably in a molten condition, and direct from the mine or from some other source of molten sulfur supply) and is heated therein, for a sufficient length of time, to a temperature sufficient to carbonize the oil. The receptacle may conveniently be contained within a furnace structure, provided with suitable fuel burners or other heating elements, and having preferably such adjuncts as heat-storing checker-work to maintain and distribute the heat generated by the combustion of the fuel. So also, as will be understood, the furnace structure may be provided with a suitable exit flue for the products of combustion, and the receptacle may be provided with a suitable take-off pipe for hydrogen sulfid and whatever vapors may be disengaged in the heating operation. Furthermore, the uniformity of the heating operation may be assured by providing the receptacle with a suitable agitating device.

We have found that the carbonizing of the oil may be carried on at temperatures

within a considerable range, provided that at the lower temperatures the heating operation is appropriately prolonged. We prefer, however, to heat the sulfur to a temperature approximating 400-430° C. and to maintain it at this temperature for about four hours. We find, that at the termination of this period of heating, the carbon resulting from the heating operation is in such a condition, in the mass, that it can be effectually removed in the subsequent stages of the operation, leaving a final product which cools to a brilliant lemon color, as will hereinafter more fully appear.

We have discovered that if, at the termination of the oil-carbonizing operation, opportunity is given the molten mass, under proper conditions, to cool to a lower temperature but without solidifying, and if this lower temperature is maintained for a sufficient length of time, the carbon will segregate out from the mass in distributed groups of aggregated particles, capable of separation by settling, filtration, or the like. The preferred range of this lower temperature is from 120° C. to 140° C., or thereabouts, and the molten mass is preferably transferred to another receptacle entirely outside of the furnace structure, and of considerably larger dimensions, so that the cooling operation may not be unduly delayed. In this second receptacle, the temperature of the mass is brought as quickly as possible to the range of 120° C. to 140° C., or thereabouts, referred to, and it is maintained at that temperature for a period of about two days. It is found that during this interval, the carbon, as above noted, segregates out from the mass in distributed groups of aggregated particles, and in such manner that it may then be separated either by settling or filtration. The addition of fullers' earth, or like material, hastens the aggregation and settling of the carbon particles.

In the accompanying drawing, is shown, in vertical section, a form of apparatus adapted to the practice of the invention, although it will be understood that the apparatus shown is but typical of other forms that may be employed for the same purpose.

In the drawing, A represents a furnace within which is sustained a receptacle B for the sulfur, said receptacle having a suitable

discharge pipe as shown. The receptacle B is provided with a cover *b*, a valved inlet pipe *c* for the admission of the molten sulfur and an exit flue *d* for the escape of hydrogen sulfid or any other vapors given off during the operation. The furnace A is provided with any suitable exit flue *f* for the products of combustion and may be heated by a fuel injector burner, indicated by *e*, or the like. *h* indicates suitable heat-storing brick-work serving as a heat storer and distributer; and *i* indicates a rotary paddle or the like whose shaft *m* is driven from any suitable source of power as, for instance, by means of the band wheel and belt shown.

The mined sulfur to be treated is supplied to the receptacle (preferably in liquid form, and direct from the mine or from a suitable supply tank) through the pipe *c* or its equivalent, the furnace and receptacle *b* having been suitably preheated. The sulfur is then brought to a sufficient temperature to carbonize the oil contained therein and is maintained at that temperature for a corresponding period of time,—dependent upon the amount of oil present in the sulfur, and the temperature employed.

As hereinbefore indicated, if the temperature of the sulfur is raised to a range of from 400 to 430° C. about four hours will usually be required to complete the desired carbonization of the oil. At lower temperatures, a correspondingly longer period of time will be required, as will be evident and as may be determined by test samples taken. A thermometer *t* is intended to afford an indication of the prevailing temperature, for the information and guidance of the operator.

At the termination of the carbonizing operation the molten sulfur containing the carbon is transferred to the vessel C provided with a heating jacket D for the circulation of steam or other heating fluid adapted to maintain the temperature of the mass at from 120° to 140° C. or thereabout. A thermometer *k* indicates the temperature.

In the vessel C, the material is maintained molten, preferably at the temperature range referred to, for a sufficient period to permit the small particles of carbon to aggregate into larger particles, which usually requires a period of about two days or more. Thereupon the separation of the sulfur and carbon can be effected by settling (aided if desired by the addition of fullers' earth, or the like), but more speedily by sand filtration. Thus, the mass, while still in the molten condition may be transferred through the valved pipe *n* to the vessel D containing a body of filtering sand *p*, through which the molten sulfur will pass, freely taking its exit through the pipe *s* and leaving the separated particles of car-

bon on the top of the filter bed. The sulfur thus obtained is free from oil and also from carbon, and is thus obtainable in the form of a product of a bright lemon color and of a quality at least equal to that of refined sulfur as found on the market at the present time.

It will be noted that we have shown said filter as provided with a steam jacket D' which may, in some instances, be usefully employed for the purpose of increasing the rapidity of flow of the sulfur through the filter and for preventing clogging thereof. So also, it may be desirable, as indicated in the drawing, to provide the conduit *a* with a power-driven endless screw, or the like, for hastening the flow of sulfur through said conduit if it should become sluggish. Above the screw, however, the conduit *a* will be provided with a cut-off valve *x* as shown.

What we claim is:

1. The method of refining mined sulfur containing oil, which comprises carbonizing the oil by maintaining a molten body of the sulfur containing it at an oil-carbonizing temperature until the desired carbonization has been effected, and then cooling the body of sulfur to a temperature above the melting point of sulfur and holding the body of sulfur at this lower temperature for a sufficient length of time to permit the segregating out of the carbon; substantially as described.

2. The method of refining mined sulfur containing oil, which comprises carbonizing the oil by maintaining a molten body of the sulfur containing it at a temperature varying from about 400° C. to 430° C. until the desired carbonization has been effected, and then holding the temperature of the body of sulfur above its melting point for a sufficient length of time to permit the segregating out of the carbon; substantially as described.

3. The method of refining mined sulfur containing oil, which comprises carbonizing the oil by maintaining a molten body of the sulfur containing it at a temperature ranging from about 400° C. to 430° C. until the desired carbonization has been effected, then holding the temperature of the body of sulfur at a range of about 120° C. to 140° C. for a sufficient length of time to permit the particles of carbon to collect in small aggregations throughout the mass and separating the carbon and sulfur; substantially as described.

4. The method of refining mined sulfur containing oil, which comprises carbonizing the oil by maintaining a molten body of the sulfur containing it at a temperature ranging from about 400° C. to 430° C. until the desired carbonization has been effected, then holding the temperature of the body of sul-

- fur at a rang of about 120° C. to 140° C. for a sufficient length of time to permit the particles of carbon to collect in small aggregations throughout the mass, adding fullers' earth to hasten such aggregation and separating the carbon and sulfur; substantially as described.
5. The method of refining mined sulfur containing oil, which comprises carbonizing the oil by maintaining a molten body of the sulfur containing it at an oil-carbonizing temperature until the desired carbonization has been effected, then cooling the body of sulfur to a temperature above the melting point of sulfur and holding the body of sulfur at this lower temperature for a sufficient length of time to permit the segregating out of the carbon, and passing the body of sulfur while still molten through a filter which is impervious to the segregated carbon; substantially as described.
- 10
6. The method of refining mined sulfur containing oil, which comprises carbonizing the oil by maintaining a molten body of the sulfur containing it at an oil-carbonizing temperature until the desired carbonization has been effected, then lowering the temperature of the body of sulfur to a point above the melting point of sulfur and maintaining the body of sulfur at this lower temperature for a relatively much longer period than at said oil carbonizing temperature and thereby causing the segregating out of the carbon; substantially as described.
- 15
- In testimony whereof we affix our signatures.

RAYMOND F. BACON.  
HAROLD S. DAVIS.